

## 1

2,938,777

## GASOLINE FUEL COMPOSITION

Thomas F. Banigan, Jr., Walnut Creek, Calif., assignor to  
Tidewater Oil Company, a corporation of Delaware

No Drawing. Original application Apr. 19, 1956, Ser. No. 579,171, now Patent No. 2,853,530, dated Sept. 23, 1958. Divided and this application Feb. 19, 1958, Ser. No. 718,108

## 2 Claims. (Cl. 44—77)

This invention relates to a fuel for internal combustion engines containing an additive, whereby cleaner operation is obtained. This application is a division of Serial No. 579,171 filed April 19, 1956, wherein the gasoline additive itself and the method for its preparation are claimed. Said application issued September 23, 1958 as Patent Number 2,853,530.

One object of the invention is to provide a cleaner fuel for internal combustion engines, such as automobile engines. Progress in the automobile industry has resulted in the development of gasoline engines of increasingly higher compression pressures, requiring gasoline fuels with correspondingly higher anti-knock properties or "octane rating." Modern refiners in an effort to obtain adequate yields of high octane gasoline are resorting to the newer processes of catalytic cracking, catalytic reforming and polymerization, and delayed or fluid coking. The stocks from such processes can provide the desired octane rating, but unfortunately such stocks often contain unstable components which tend to form deposits in critical parts of the induction system such as the carburetor throat, intake manifold and intake valve ports. Heretofore, use of gasolines made from these stocks has commonly resulted in fouling such parts in a few thousand miles, especially where the cars have been subjected to city driving or other low-output types of use. As these deposits accumulate, the engine's idling becomes labored and uneven, and stalling often results. Deposits also form in the combustion chamber, and, as a result of the various deposits, the engine exhibits a loss of power, gives poor gasoline mileage, and eventually requires higher octane fuel.

These conditions are the result of unstable constituents in the fuel reacting under the influence of heat, oxygen, blowby gases and exhaust gases. While it might be possible to refine all unstable constituents out of the fuel, it is generally not feasible to do so. The deposit-forming tendency at times is accentuated when lead tetraethyl and dyes are present.

Many substances have been tried as gasoline additives in attempts to solve the above problems, but the results have fallen far short of expectations. Various detergents and gum solvents have been mixed with the gasoline in an attempt to prevent the formation of deposits. Many volatile polar compounds which should be capable of dissolving the deposits have been tried, unsuccessfully. Acetone and other ketones, tetrahydrofuran, oxydipropionitrile, iminodipropionitrile, morpholine, quinoline, cyclohexanone, nitrobenzene, di-tertiarybutyl-paracresol, polypropylene glycols and ammonium mahogany sulfonate are among the compounds tried. None of these appear to give improvement in overall engine cleanliness; some of them decrease deposits in one part of the engine only to transfer what they pick up to other parts of the engine, where they are redeposited. Some of these contribute to the deposits in the carburetor and on the valve stems; some cause ring sticking; and some increase overall dirtiness throughout the engine.

## 2

Other types of gasoline additives, such as tricresyl phosphate, do not reduce the engine deposits but rely instead on chemical change of the deposits in the combustion chamber to suppress preignition usually resulting from such deposits. This type of additive is of no value in preventing induction system deposits or piston-ring sticking.

An important object of this invention is, therefore, to provide a fuel that has substantially less tendency to build up intake manifold and engine deposits.

Another object of the invention is to obtain cleaner carburetion by providing a fuel that does not foul up the carburetor.

Another object of the invention is to prevent loss of power by reducing the tendency for piston-ring sticking.

Other objects and advantages of the invention will appear from the following description.

Bis[2-(1-methoxyisopropoxyisopropoxy) ethyl] ether has the formula  $\text{CH}_3(\text{OC}_2\text{H}_5\text{CH}_3)_2\text{O}(\text{CH}_2)_2\text{O}(\text{CH}_2)_2(\text{OC}_2\text{H}_5\text{CH}_3)_2\text{OCH}_3$ . This substance is claimed in application Serial No. 579,171 filed April 19, 1956, and its preparation is therein described and claimed. Said application issued September 23, 1958 as Patent Number 2,853,530.

25 The polyether is a colorless, slightly viscous liquid. It is completely miscible with organic solvents such as benzene, xylene, pentane, octane, iso-octane, ethyl alcohol and ethyl ether, but only partially soluble in water. The compound is stable, as shown by the fact that one sample, 30 stored for eight months, in a clear bottle, showed no change in color or properties. The compound is inflammable, burning readily with no smoke and essentially no carbon residue.

35 The polyether has approximately the following physical properties:

Boiling point, °C.:

at 770 mm. (atmos. press.) 185  
at 30 mm. 107

40 Freezing point, °C. glass below -60

Refractive index,  $n_{D}^{20}$  1.4214

Density,  $d_{4}^{20}$  0.9527

Molecular refraction:

Experimental (Lorentz & Lorenz) 97.5

45 Theoretical (Auwers & Eisenlohr) 96.8

Viscosity:

Saybolt seconds @ 100° F. 34.3

Centistokes @ 100° F. 2.46

Carbon residue, % less than 0.01

50 Solubility in water @ 25°C., g./100g. 12

Performance tests have shown that the present invention produces substantial improvement in engine cleanliness, as compared to the same fuel not containing the additive. The test procedure (designated hereinafter as "40-E" procedure) involves a 40 hour engine run on a dynamometer under conditions chosen to correlate, on an accelerated scale, with field performance. In this test a 216.5 cubic-inch, six-cylinder Chevrolet engine is run continuously for forty hours at a speed of 1900 r.p.m. (plus or minus 25 r.p.m.) under an engine load of 36 B.H.P. (plus or minus 1 B.H.P.). The jacket coolant inlet temperature is kept at 155° F. minimum, the jacket coolant outlet temperature is kept within two degrees of 170° F., and the crankcase oil temperature is kept within two degrees of 190° F. The air-fuel ratio is 14.5 (plus or minus 0.5) to 1. The spark advance is 35° (plus or minus 3°). The spark plug gap, ignition cam angle, valve clearance, exhaust back pressure and other similar conditions are also maintained at predetermined values. Before the test, the engine is disassembled and cleaned, and a new set of piston rings is installed. The

engine is given a standard two-hour break-in before the actual test is begun.

After the test run of 40 hours, the engine is dismantled and inspected, and is rated on ten items, as follows:

- (1) Piston skirt varnish rating.
- (2) Cylinder wall varnish rating.
- (3) Intake valve stem deposit rating.
- (4) Intake valve tulip deposit rating.
- (5) Intake port deposit rating.
- (6) Overall engine sludge rating.
- (7) Overall engine varnish rating.

On these first seven items, the rating runs between 0 for dirty to 10 for clean.

(8) Corrosion or rust rating (10 for none, 9 for light, 8 for medium, and 7 for heavy corrosion).

(9) Stuck ring rating (10, minus 0.5 demerit for each 90° of ring stuck in the groove).

(10) Tight ring rating (10, minus 0.5 demerit for each tight ring).

A perfectly clean engine will thus rate 100. A total rating of 85 is considered acceptable if the piston skirt varnish is 7.5 or better.

The gasoline employed in the tests discussed herein-after for illustration was composed of about 50% mixed thermal naphtha having about 95°-400° F. boiling range, about 20% light straight-run naphtha having 95°-250° F. boiling range, about 25% heavy cracked (catalytic) naphtha having 270°-400° F. boiling range, and about 5% of light natural gasoline. It contained as additives about 1.75 ml. per gallon of tetraethyllead and an amine inhibitor in normal amounts. It analyzed 0.11% sulfur. Gum was present at about 2 to 5 mg. per 100 ml. in the ASTM test and the copper dish test showed about 16-26 mg. of gum per 100 ml. The gasoline had the following volatility specifications: 10% evaporated at 134°-150° F., 50% at 244°-250° F., and 90% at about 360° F. The approximate composition of the gasoline was:

|                            | Percent     |
|----------------------------|-------------|
| Paraffins and naphthalenes | about 66    |
| Olefins                    | about 16    |
| Aromatics                  | about 18    |
| Sulfur                     | about 0.1   |
| Phenols                    | about 0.4   |
| Nitrogen                   | about 0.001 |

Table I shows the results of such tests where 0.75 cc./gal. of the new compound of this invention was used, in comparison with the same gasoline without the bis[2-(1-methoxyisopropoxyisopropoxy) ethyl] ether.

As blended into the gasoline, the new compound contained about 2% by weight of an antioxidant (phenyl-alphanaphthylamine) which had been added to assure against possible oxidation in storage and blending operations.

10

15

Table I

|                | Control<br>Gasoline | Gasoline<br>Plus Addi-<br>tive 75 gm./<br>100 gal. |
|----------------|---------------------|----------------------------------------------------|
| Overall Rating | 83                  | 86.5                                               |

Table II shows a breakdown of some of the items in the same test as Table I.

20

25

30

Table II

|                           | Control<br>Gasoline | Gasoline<br>plus<br>Additive |
|---------------------------|---------------------|------------------------------|
| Piston skirt rating       | 7.5                 | 8.0                          |
| Intake valve tulip rating | 9.0                 | 9.0                          |
| Intake valve stem rating  | 9.0                 | 9.0                          |
| Stuck ring rating         | 8.0                 | 10.0                         |
| Overall varnish           | 7.0                 | 8.0                          |
| Side pan sludge           | 7.0                 | 8.0                          |

The superior stuck-ring-rating of the gasoline containing the new additive is particularly impressive.

I claim:

35 1. A gasoline containing bis[2-(1-methoxyisopropoxyisopropoxy) ethyl] ether as an additive in amount sufficient to substantially reduce engine deposits.

30

2. A fuel according to claim 1 wherein the concentration of the additive is about 0.75 cc. per gallon of gasoline.

#### References Cited in the file of this patent

#### UNITED STATES PATENTS

|              |                  |                |
|--------------|------------------|----------------|
| 45 2,425,845 | Toussaint et al. | Aug. 19, 1947  |
| 2,563,101    | Colwell et al.   | Aug. 7, 1951   |
| 2,800,400    | Hughes           | July 23, 1957  |
| 2,807,526    | Foreman          | Sept. 24, 1957 |